

# United States Patent Office

3,689,386

Patented Sept. 5, 1972

1

3,689,386

## METHOD FOR THE SURFACE TREATMENT OF ALUMINUM ELECTRODES FOR THE ELECTROLYTIC PRODUCTION OF ZINC, AND ELECTRODES THUS TREATED

Giovanni Scacciati and Giovanni Lanfranco, Turin, Italy, assignors to Centro Ricerche Metallurgiche S.p.A., Turin, Italy

No Drawing. Filed Nov. 30, 1970, Ser. No. 93,889  
Claims priority, application Italy, Dec. 2, 1969,

25,229/69

Int. Cl. C22d 1/22; B01r 1/00; C23c 1/08

U.S. Cl. 204—114

4 Claims

### ABSTRACT OF THE DISCLOSURE

A method is disclosed for the surface treatment of aluminum electrodes for the electrolytic production of zinc substantially consisting in dipping said electrodes, before their use, into a bath comprising an aqueous solution of at least one acid selected from the class consisting of hydrofluoric acid and fluosilicic acid. The concentration of the acid in the treating bath is between 1 to 20 g./l., and the dipping time is between 5 and 500 seconds.

The present invention relates to a method for the surface treatment of the aluminum electrodes used for the production of zinc by electrolysis, in order to eliminate, or at least reduce to a minimum, the harmful effect of fluorine present in the electrolytic solution. The invention also relates to the aluminum electrodes thus treated.

It is quite well known that one of the most difficult problems in the metallurgy of zinc by electrolysis arises from the presence of fluorine in the electrolyte. In fact, when the fluorine content exceeds certain values, there occurs the phenomenon of the adhesion of the zinc deposits to the aluminum cathodes. This adhesion may be such as to make it very difficult—if not indeed impossible—to bring about the detachment of the zinc deposit; or, as it is commonly called, the stripping of the zinc deposit.

Since the greatest part of the zinc ores contains fluorine in more or less great quantities, this problem is common and always present in all the electrolytic zinc plants. Often there occur production losses and, at any rate, the control of the fluorine invariably represents a costly and difficult problem. Moreover, certain zinc ores, excellent from any other point of view but containing high percentages of fluorine, cannot be accepted for the metallurgical treatment via electrolysis.

The adhesion phenomenon is ascribed to the pickling action which the fluorine present in the electrolyte exerts on the surface of the aluminum at the starting stage of the electrolysis; that is, when said surface is not yet completely covered by the depositing zinc. The pickling action consists in destroying the oxide film that lies on the aluminum surface and which hinders the adhesion of the zinc deposit.

The phenomenon manifests itself in a different manner in different plants, depending on the electrolysis conditions, and is probably related to numerous other factors.

Therefore, so far it has been impossible to correlate the effect of the fluorine with its concentration in the electrolyte; for example, there exist plants that cannot tolerate more than 15–20 mg./l. of fluorine, and others that on the contrary operate with 200 mg./l. and more of fluorine.

In any case, a sudden increase of fluorine, resulting in fluorine contents above the customary levels, is the cause of the difficulty or impossibility of the zinc stripping operation.

2

Different proposals for eliminating the harmful effect resulting from the fluorine have been studied and applied but none so far has yielded results satisfactory in all cases. One of the most frequently used methods is that of dipping for some time the electrically insulated aluminum cathodes into the electrolytic cell. This expedient is, however, often inadequate and, at any rate, rather burdensome in as much as it disturbs the normal operation of the electrolysis and results in high labor costs.

5 Thus, an object of this invention is to provide a method for the surface treatment of aluminum cathodes such as to eliminate in all cases, or at least to reduce to a minimum, the above-cited harmful effects of the fluorine.

10 Another object of this invention is to provide a cheap method, capable of easy fulfillment, for the treatment of aluminum cathodes.

15 These, and still other objects that will appear more clearly from the detailed description that follows hereunder, are conveniently achieved by a method for the surface treatment of the aluminum electrodes for the electrolytic production of zinc; said method, according to this invention, substantially consisting in dipping said electrodes, before their use, into a bath including an aqueous solution of at least one acid selected from the class consisting of hydrofluoric acid and fluosilicic acid.

20 The dipping times may vary within wide limits, depending on the desired effect, for instance from 5 to 500 seconds. For reasons of maximum productivity, preference will be given to dipping times as short as possible.

25 Likewise, the concentration of the acid used in the treatment bath may vary within rather wide limits; thus, for instance, use can be made of a bath having an acid concentration between 1 and 20 g./l.

30 The protective action which the above-indicated treating bath develops on the aluminum electrodes, thus avoiding or reducing to a minimum the etching by the fluorine contained in the electrolytic solution, and the consequently high adherence of the zinc deposited on said electrodes, may be explained in the following way, according to a hypothesis believed to be correct but not to be taken as limiting the invention.

35 The dipping of the aluminum electrode into the bath containing the acid causes the formation on the surface of the aluminum of a thin layer of salts of the aluminum fluoride type or of the aluminum fluosilicate type, depending on the acid used, said salts being more or less hydrated. These salts show a greater resistance than the aluminum oxide originally existing on the surface of the electrode to the aggressive action of the fluorine contained in the electrolyte.

40 The thin film of salts sets up a kind of cushion between the aluminum and the zinc forming thereon during the electrolysis of the zinc solution, thereby hindering the direct contact between the two metals and thereby facilitating their subsequent separation.

45 It should be noted that it is not necessary to repeat the dipping into the acid bath for each electrolytic cycle; the effect of one treatment may be enough for 2–3 successive cycles.

50 The corrosion of the aluminum cathode which is caused by the treating method according to this invention is quite irrelevant. In fact, it has been found that for an aluminum electrode having 1 sq. m. of total immersed surface and for a treatment every 48 hours, in one year a loss of about 10 g. of aluminum occurs based on a total weight of 5–6 kg. of immersed portion. Thus, the treatment does not significantly affect the normal average life of the aluminum electrodes.

55 In industrial practice, after each electrolytic cycle (generally during 24 or 48 hours) the set of electrodes is carried to the manually or automatically operating stripping station, where the zinc deposits are stripped from the

aluminum cathodes; thereafter these latter are washed with water and again arranged in electrolytic cells.

The dipping into the treatment bath according to this invention is made after the stripping and before the water-washing. Since the dipping treatment only takes a few seconds or at most a few ten seconds, it affects the electrolytic cycle to a quite negligible extent.

In order still better to illustrate this invention, a few examples are now given. These examples were obtained from a series of tests performed by feeding 4 industrial electrolytic cells, arranged in cascade, with the electrolyte for zinc addition with an established quantity of fluorides. Each cell had 6 aluminum cathodes. The average operational conditions were:

Feed into 1st cell:  $Zn=80$  g./l.;  $H_2SO_4=90$  g./l.;  
Outflow from last cell:  $Zn=60$  g./l.;  $H_2SO_4=120$  g./l.;  
Temperature:  $40^\circ C.$ ;  
Current density: 500 amp./sq. m.

#### EXAMPLE 1

The feeding solution contained 50 mg./l. of fluorine. Three cathodes of each electrolytic cell, after having been washed with water, were treated, according to this invention, by dipping them for 60 seconds into a solution of 2 g./l. of fluosilicic acid.

After the treatment the cathodes were washed with a jet of water and subsequently employed in the electrolysis.

The stripping of the zinc deposited on the thus pre-treated cathodes was easy.

The stripping of zinc from the non-pre-treated cathodes of the same cells was very difficult if not impossible.

#### EXAMPLE 2

The feeding solution contained 50 mg./l. of fluorine. Three cathodes of each cell, after having been washed with water, were treated, according to this invention, by dipping them for 60 seconds into a solution of 1.5 g./l. of hydrofluoric acid.

After the treatment the cathodes were washed with a jet of water and subsequently employed in the electrolysis.

The stripping of the zinc deposited on the thus pre-treated cathodes was easily done.

The stripping from the non-pre-treated cathodes of the same cells was very difficult, if not impossible.

What is claimed is:

1. A method for the surface treatment of aluminum electrodes for the electrolytic production of zinc wherein said electrodes, before their use, are dipped into a bath consisting of an aqueous solution of at least one acid selected from the class consisting of hydrofluoric acid and fluosilicic acid, and thereafter using said electrode as a cathode in a cell during the electrolytic production of zinc.

2. A method according to claim 1, wherein the concentration of the acid in the treating bath is between about 1 and 20 g./l.

3. A method according to claim 1, wherein the dipping time in the treating bath is between about 5 and 500 seconds.

4. An aluminum electrode for the electrolytic production of zinc, the surface of which is covered by a thin layer of a salt selected from the class consisting of aluminum fluoride and aluminum fluosilicate.

#### References Cited

##### UNITED STATES PATENTS

|           |         |                 |       |          |
|-----------|---------|-----------------|-------|----------|
| 3,495,457 | 1/1950  | Jacobs          | ----- | 204—281  |
| 2,213,263 | 9/1940  | Thompson et al. | ----- | 148—6.27 |
| 2,391,522 | 12/1945 | Slunder         | ----- | 148—6.27 |
| 2,032,897 | 3/1936  | Tanner          | ----- | 148—6.27 |
| 2,825,697 | 3/1958  | Carroll et al.  | ----- | 148—6.27 |

#### OTHER REFERENCES

Kirk, R. and Othmer, D. F. Encyclopedia of Chemical Technology, vol. 15, pp. 258—9, 1956. The Interscience Encyclopedia, Inc., N.Y.

JOHN H. MACK, Primary Examiner

R. J. FAY, Assistant Examiner

#### U.S. Cl. X.R.

117—130; 148—6.27; 204—12, 281, 290 F